

No. 669,952.

Patented Mar. 12, 1901.

W. BRINTON.

## MOLD FOR STEEL CASTINGS.

(Application filed Dec. 5, 1900.)

(No Model.)

2 Sheets—Sheet 1.



Fig: 1.



Fig: 2.



WITNESSES:

C INVENTOR  
Walter Birdstone,  
BY Crosby Gregory

**ATTORNEYS.**

No. 669,952.

Patented Mar. 12, 1901.

W. BRINTON.

MOLD FOR STEEL CASTINGS.

(Application filed Dec. 5, 1900.)

(No Model.)

2 Sheets—Sheet 2.



Fig. 3.



Fig. 5.



WITNESSES:

Edward G. Allen.  
Adolph C. Haase.

INVENTOR

Walter Brinton,  
BY Shirley Gregory.

ATTORNEYS.

# UNITED STATES PATENT OFFICE.

WALTER BRINTON, OF HIBRIDGE, NEW JERSEY, ASSIGNOR TO TAYLOR  
IRON & STEEL COMPANY, OF SAME PLACE.

## MOLD FOR STEEL CASTINGS.

SPECIFICATION forming part of Letters Patent No. 669,952, dated March 12, 1901.

Application filed December 5, 1900. Serial No. 38,850. (No model.)

To all whom it may concern:

Be it known that I, WALTER BRINTON, a citizen of the United States, and a resident of Highbridge, in the county of Hunterdon and State of New Jersey, have invented an improvement in Molds for Steel Castings, of which the following description, in connection with the accompanying drawings, is a specification, like letters on the drawings representing like parts.

In casting steel, and particularly steel projectiles, it has heretofore been the practice to use molds having a metallic lower portion, such as iron or steel, in order to rapidly chill the molten steel contacting with the metallic portion, the upper portion of such mold being constructed of sand or having a sand lining, so that the molten metal in that part of the mold will cool more gradually. When casting a steel projectile, for instance, in such a mold, there is a great tendency to crack and set up highly-objectionable strains in that portion of the projectile at the junction of the chill and sand, such tendency being due to the more rapid contraction of the part of the metal cast in the metallic chill.

This invention has for its object the avoidance of such defects, preventing the formation of cracks, and the setting up of objectionable strains, and I attain such object by so constructing the mold that an intermediate region or zone is provided between the chill and the non-chilling part of the mold, so that the rate of cooling of the casting adjacent thereto gradually changes from a comparatively rapid rate at the chilled part to the relatively slower rate at the non-chilled part of the casting.

Figure 1 is a horizontal section on the line  $xx$ , Fig. 2, of a mold, illustrating one embodiment of my invention. Fig. 2 is a vertical sectional view thereof, the upper part of the mold being broken away. Fig. 2<sup>a</sup> is a detail view similar to Fig. 1, showing the upper part of the chill with the sand omitted from the intermediate part of the mold. Fig. 3 is a vertical sectional view of a modification to be described. Fig. 4 is a top or plan view of a modification of the chill and intermediate

zone, and Fig. 5 is a vertical section of the chill shown in Fig. 3.

Inasmuch as my invention is particularly adapted for casting projectiles I have herein shown the molds as constructed and arranged for such use; but it will be manifest to those skilled in the art that by suitably changing the shape or configuration of the molds other articles may be cast in accordance with my invention.

Referring to Figs. 1, 2, and 2<sup>a</sup>, the chill  $a$  of the mold is made of iron or steel and in the present instance receives the molten steel which is to form the point and head of the projectile, so that such parts shall be rapidly cooled or chilled by contact with the metal, and the top of the chill is laterally enlarged, as at  $a'$ , to provide a firm support for the non-chilling portion or member of the mold, comprising a box or flask  $f$ , having a sand lining  $e$ , the annular rib  $f'$  at the bottom of the flask entering the correspondingly-recessed part  $a^2$  in the top of the chill. An internal annular recess  $c$  is formed at the top of the chill, the bottom  $c^2$  of such recess being shown as scalloped, serrated, or corrugated, the structure being very clearly shown in Fig. 2<sup>a</sup>, in which the upper part of the chill is shown with the sand removed.

In using the mold sand is filled into and packed in usual manner in the recess  $c$ , its top being smoothed off to form a closed joint with the bottom of the sand lining  $e$ , (see Fig. 2,) so that a series of finger-like portions  $d$  of sand are presented. The intermediate portion of the mold between the bottom of the non-chilling portion and the main part of the chill will therefore be composed of alternating juxtaposed portions of sand and metal, which come in contact with the cast metal between the chilled and the non-chilled portions thereof, the effect to such intermediate zone being to reduce the rapidity of cooling of the adjacent part of the casting, such rate decreasing from the comparatively rapid rate at the full metallic part of the chill to the relatively slower rate at the bottom of the non-chilling member of the mold, such retardation of the cooling preventing in the

casting a sudden transition from rapid to slow cooling, with the attendant formation of cracks, openings, or other defects, or the setting up of highly objectionable internal strains in the casting.

In Fig. 3 the chill *g* is constructed in usual manner, except that the top thereof within the annular seat *g'* for the non-chilling body portion or flask *f* is scalloped, corrugated, or serrated, as at *g''*, (see also Fig. 5,) and the sand lining *e* of the body portion of the mold is carried down to and between the corrugations, as at *e''*, Fig. 3, so that alternating and juxtaposed portions of metal and sand are presented at the intermediate portion of the mold for the purpose hereinbefore set forth.

The construction of the chill is very clearly illustrated in Fig. 5.

In Fig. 4 I have shown in top or plan view a modification wherein the upper part of the wall of the chill *k* is formed with internal ribs or corrugations, as at *k'*, extended in the direction of the length of the depth of the chill and gradually increasing in size toward the top of the chill. Sand is packed into the corrugated or ribbed portion, as at *k''*, and faced to the configuration of the interior of the chill, so that graduated portions of alternating sand and metal form the intermediate portion of the mold, the thickest part of a sand portion coming next to the thinnest part of a metal rib or corrugation, and vice versa.

By the use of molds such as hereinbefore described the contraction of the cast-steel takes place gradually at the intermediate portion of a mold, the rapidly-cooling portion of the casting below it and within the chill blending or grading into the more slowly cooling part in the body portion of the mold,

so that the resulting casting is free from the 40 defects hereinbefore referred to.

Having fully described my invention, what I claim, and desire to secure by Letters Patent, is—

1. A mold for producing castings, comprising a metallic portion to chill the contained metal, a sand portion to permit more gradual cooling of the metal adjacent thereto, and an intermediate zone composed of continuations of the metallic and sand portions of the mold 45 in juxtaposition, and both exposed to contact with the incoming molten metal, and arranged to decrease the rate of cooling of the adjacent metal of the casting from the chill to the sand part of the mold.

55 2. A mold for producing castings, comprising a metallic portion to chill the contained metal, a sand portion to permit more gradual cooling of the metal adjacent thereto, and an intermediate zone composed of alternating 60 portions of sand and metal.

3. A mold for producing castings, comprising a metallic portion to chill the contained metal, a non-chilling portion to permit more gradual cooling of the casting adjacent thereto, and an intermediate portion formed of overlapping and alternately arranged and exposed extensions of the chilling and non-chilling portions of the mold, to prevent sudden variations in the cooling of the intermediate portion of the casting.

65 In testimony whereof I have signed my name to this specification in the presence of two subscribing witnesses.

70 WALTER BRINTON.

Witnesses:

BEN. F. ROBBINS,  
R. D. STRUBLE.